

## UNITED STATES PATENT OFFICE

LESTER KIRSCHBRAUN, OF LEONIA, NEW JERSEY

## AQUEOUS DISPERSIONS AND PROCESS OF MAKING SAME

No Drawing.

Application filed October 6, 1927. Serial No. 224,526.

This invention has relation to the production of aqueous dispersions of materials normally immiscible with, or insoluble in, water, and is more particularly concerned with water 5 dispersions of solid or semi-solid bitumens such as asphalt and the like.

In one of the methods which has met with considerable success for producing this type 10 of dispersion, the solid or semi-solid bitumen or other material to be dispersed is subjected, while in fluid condition, to a severe and rapid agitating action in the presence of a highly viscous mass comprised, generally, of material undergoing dispersion together with a certain 15 quantity of material functioning as a dispersing medium. In actual commercial practice, a large bulk supply of finished product is constantly maintained in the apparatus of which the agitating mechanism forms a part, 20 and the material to be dispersed is fed to this apparatus in fluid condition while a separate stream comprising an aqueous suspension of dispersing medium is simultaneously led into the mass undergoing agitation, suitable provision being made for continuously or intermittently withdrawing the dispersed material 25 from the apparatus.

In order to produce dispersions of this character which shall be capable of admixture 30 with electrolytes without destroying the character of the product as a dispersion, it is essential to employ as the dispersing agent materials or combinations of materials which are relatively inert chemically and incapable 35 of entering into any reaction with or being reacted upon by the specific electrolyte which may be proposed for admixture with the product. It will be appreciated in this connection, where the dispersing agent is such 40 that a specific electrolyte may react therewith and impair or destroy its dispersive or protective properties, that under such conditions the dispersive agent may no longer be able to function, with the result that the aqueous 45 dispersed condition of the system is destroyed and the dispersion is then said to be broken.

For the purpose of providing dispersive media which shall be relatively inert to such action, and which possess other desirable advantages, there have been employed certain

organic and inorganic powders, insoluble in, though readily wetted with, water and capable of swelling or being treated so as to swell more or less and assume a plastic condition in the presence of water. Of this class of materials, clays, metallic silicates and oxides, casein and other proteins, starch, etc. are examples, although clays are generally preferred and have found extensive application in this field, since they are comparatively inexpensive and possess to the largest extent the inertness and other properties necessary to produce the desired product.

It has been found that certain of these mineral powder types of dispersive media, for instance, certain kinds of clays and metallic oxides, are sometimes deficient in suspending power, so that while they are capable of exercising their function in the production of the dispersions, they are, on the other hand, 65 more or less unable to effect a sufficiently fine dispersion to retain the entire mass of dispersed particles in suspension in the aqueous phase over long periods of time, with the result that the particles gradually settle out to 70 a greater or less extent.

Emulsions made with various types of emulsifying agents in which the dispersed particles, among other conditions, are not sufficiently fine, are prone to settle out. It is 80 sometimes difficult to secure fine dispersion either because of the type of emulsifying agent used, the viscosity of the mass, temperatures, character of equipment, or the like. The purpose of the present invention is to 85 treat dispersions which have been made, or are being made under such unfavorable conditions as might impair their suspensibility, in such a manner as to render them suspensible despite their large particle size.

The present invention is particularly concerned with dispersions made with dispersive media which are open to the foregoing objections, and is directed to methods of treatment whereby such dispersions may be converted 95 into products of improved and relatively permanent suspensibility.

The invention further comprehends methods for treating dispersive media of the aforesaid character and which ordinarily 100

give rise to non-suspendable products in such manner as to render them capable of producing more highly suspendable dispersions.

In its broadest aspect, the invention proceeds upon the principle of forming a cellular or gel-like structure in the dispersed product. The invention is embodied in various modes of procedure which are hereinafter to be described in greater detail, and in accordance 10 with which the gel formation in the product is derived by the employment of substances which react with one another to produce what are termed silica gels. It should be understood, however, that this is merely one type 15 of gel which has been found to be practical in carrying out the principles of the invention, and that the broad concept is not to be regarded as restricted or limited to this particular type of gel.

20 One convenient method by which silica gels may be formed is to treat an aqueous solution of sodium silicate with ammonium chloride or hydrochloric acid whereby there is precipitated a highly gelatinous mass composed 25 largely of silicic acid. The character of the gel thus formed depends upon the concentration of the silicate solution employed as well as that of the reagent with which the silicate is treated to form the silica gel.

30 It seems to be characteristic of silica gels as thus produced that when they are agitated or stirred, they are disrupted into more or less grainy particles distributed in irregular and non-homogeneous fashion throughout 35 the mass, and, particularly when the silicate concentration has been relatively low, a large quantity of free water appears after the gel has been agitated. With high concentrations of silicate and more rigid gels, the gel is 40 not destroyed although it may be broken up and the separate portions of the rigid gels subsequently coalesce upon standing. On the other hand, it has been observed that where silica gels are formed, in dispersions of 45 the type here referred to, the gelled dispersion thereby produced, possesses the unique property of being able to regain its gel character upon standing quiet for a short time subsequent to having had the gel formation thereof converted to liquid as by stirring 50 or otherwise. This phenomenon, i. e., to liquefy by stirring and reassume gel structure on standing, does not occur with silica gels, per se, made from aqueous solutions of equal 55 sodium silicate concentration.

60 By virtue of this peculiar behavior of dispersions having gels formed therein, it becomes possible to prepare such dispersions and rely upon the gelled condition of the aqueous continuous phase to maintain the dispersed particles in suspension, even after the product has been subjected to stirring action or similar influence whereby the gel is 65 temporarily dissipated, since upon permitting

a short time, the gelled condition is restored and can then exert its function in retaining the particles in suspension.

In carrying out the invention in accordance with the foregoing principle, it is found 70 that the concentration of sodium silicate and the pH value determines the degree of gelling and the rapidity with which the gelling action takes place. Generally, the lower the hydrogen ion concentration of the gelled dispersion, the greater the concentration of sodium silicate must be, and vice versa. 75

In one mode of carrying out the invention, there may first be prepared an aqueous dispersion of bituminous material such as steam refined Mexican asphalt having a melting point of, say 100° to 200° F., more or less, using ordinary brick making clay as the dispersing agent. This dispersion may be effected in any desired manner, for instance, in accordance with the methods disclosed in United States Letters Patent No. 1,302,810. Such dispersion may be composed of, say, 50-55% of the asphalt, 5 to 10% of clay dispersing agent, and the balance water. To a 90 suitable quantity of the dispersion thus produced, there may be added about 1.8%, more or less, by weight of commercial 44% sodium silicate solution. Hydrochloric acid in quantities sufficient to bring the hydrogen ion concentration to a pH value say, 3.0 to 3.3, more or less, may be then added to the silicate treated dispersion, with the result that a gel formation takes place in situ in the dispersion, and this gel structure exerts a protective action on the dispersed particles and serves to retain them in relatively permanent suspension. 95

100 The invention may also be carried out by a somewhat modified procedure in which the silicate treatment is applied to the dispersing agent prior to effecting the dispersion therewith. In this procedure, it is preferable that the concentration of silicate and acid be such that no gelling takes place in the aqueous 110 suspension containing the dispersing agent and silicate, since too severe gelling action in the dispersive media will obviously interfere with the dispersing action which is to be effected therewith. The concentration may 115 be therefore preferably adjusted so as to delay the formation of the gel until after the dispersing action has been completed. Accordingly, illustrating such a procedure, say 20 parts, more or less, of brick making 120 clay may be mixed with, say, 100 parts of water containing, say, 5 parts, more or less, of the commercial 44% sodium silicate solution. Sufficient hydrochloric acid may be then added to the mixture to bring the hydrogen ion concentration thereof to a pH value of, say, 2.0 to 2.3, more or less. At this pH value, substantially no gelling takes place but the aqueous suspension is of a sirupy 125 consistency which functions efficiently as the 130

dispersive media. Any bitumen-type base, such as asphalt, may be dispersed with this media in the manner set forth in the said patent. The dispersion so produced will increase in pH value due to the dispersed asphalt, but preferably should be brought to a final pH value of, say, 3.0 to 3.5, more or less, if it is not already of such value, in order to obtain the gelling action above described and so that the water-free film of the product may be resistant to the action of water and irreversible. Upon allowing this heavy product to stand, it assumes a gel condition, and it may be beaten or stirred out, if necessary, to convert the mass into a viscous body of desired consistency, and thereafter, by permitting the beaten out mass to remain quiescent, the gel will reform in the mass, as already described, and function to maintain the product in suspension.

Should it be necessary or desirable to thin out the heavy dispersion as withdrawn from the dispersing apparatus, this may be done with water, or with an aqueous solution of sodium silicate and hydrochloric acid, although in order to favor the ready formation of the silica gel in the dispersed mass, it is preferable to employ the sodium silicate solution containing the hydrochloric acid. For this purpose, and to thus thin out the dispersion made as above described with the silicate-treated clay dispersing media, there may be added to the heavy dispersion an aqueous solution composed of about 2.2% sodium silicate, more or less, acidified with hydrochloric acid to a pH value of about 3.0, more or less. This solution may be employed in such quantities as are necessary to bring about the desired fluidity in the product.

As a further illustration of the foregoing procedure with another material possessing relatively poor suspending power, a Kentucky ball clay may be employed as the dispersing agent. With this substance, however, it has been found that for more successful results it is necessary to use lower concentrations of the sodium silicate, and also to operate at a pH value different from the 3.0 to 3.5 value used in connection with the preceding clay, since at this value with the Kentucky clay it is more difficult to carry on the dispersing action and the gel formed is too rigid and does not beat out easily to the desired body and viscosity. Hence, in order to disperse a material such as Mexican asphalt, the dispersive media may preferably comprise 20 parts, more or less, of the Kentucky clay and 100 parts of water containing approximately 3 parts, more or less, of the commercial 44% sodium silicate solution, and acidified with hydrochloric acid to a pH value of, say, 6.0 to 6.5, more or less. With such dispersive media, the asphalt may be dispersed more readily and the gel formed in the dispersion may be easily beaten or

stirred out to a homogeneous body of desired consistency, the gel being subsequently reformed upon allowing the product to remain quiet, and as long as the gelled condition exists in the product, the dispersed particles are enabled to remain in suspension. The product as thus produced is capable, without any further treatment for the modification of its pH value, of drying to a film which is highly resistant to permeation by water.

Ammonium chloride and other equivalent materials may be used instead of hydrochloric acid, if desired.

By the use of the term "gel" or "gelled" in the claims I intend to define an emulsion possessed of the unique property of being able to regain its "gelled" character by standing quiet for a short time subsequent to having had the "gelled" formation thereof converted to liquid with a slight amount of stirring and without the use of a diluent or substantial quantities thereof.

I claim as my invention:

1. An aqueous gelled dispersion of a waterproofing material, the aqueous phase containing silica in "gelled" form.

2. An aqueous gelled dispersion of a waterproofing material, the aqueous phase being in the form of a "gel".

3. A product of the character described, comprising a waterproofing material dispersed in a "gelled" aqueous vehicle.

4. A product of the character described, comprising a dispersion, the continuous phase of which is in the form of a "gell", the internal phase of said dispersion comprising a waterproofing material.

5. A product of the character described, comprising a waterproofing material dispersed in an aqueous vehicle, said product being characterized by its ability to "gel" on standing.

6. A gelled product comprising a waterproofing material dispersed in an aqueous vehicle, the "gel" condition of said product being dispelled by agitating action, said product being characterized by its ability to return to the "gel" condition upon standing quiet after being subjected to such action as has been sufficient to dispel the "gel" condition thereof.

7. A product of the character described, comprising a waterproofing material dispersed in water, and containing substances for causing a "gelled" formation in the aqueous phase thereof.

8. A product of the character described, comprising a water-proofing material dispersed in water, and containing substances for causing the formation of silica "gel" in the product.

9. In the production of dispersions, the dispersed waterproofing particles whereof tend to settle out of suspension, the step which

comprises forming a "gel" in situ in the dispersion.

10. In the production of dispersions, the dispersed waterproofing particles whereof 5 tend to settle out of suspension, the step which comprises forming a silica "gel" in situ in the dispersion.

11. The method of treating aqueous dispersions whereby to increase the ability of 10 the dispersed waterproofing particles thereof to remain in suspension, which comprises combining with the aqueous dispersion a material capable of inducing a "gel" formation in the aqueous phase thereof.

15. 12. The method of treating dispersions whereby to increase the ability of the dispersed waterproofing particles thereof to remain in suspension, which comprises combining with the dispersion a material capable 20 of inducing a silica "gel" formation in the dispersion.

13. In the production of dispersions, the steps which comprise combining with a mineral powder dispersing media, substances 25 capable of producing a "gel" formation in the dispersion, and effecting dispersion of a waterproofing material, with said combined mixture.

In testimony whereof I affix my signature.  
30 LESTER KIRSCHBRAUN.

35

40

45

50

55

60

65